

1,466,738

Sept. 4, 1923.

C. S. MORSE

METHOD AND MEANS FOR BILLET CASTING

Filed July 2, 1921.



Fig. 2.

Fig. 1.

Inventor:  
Charles S. Morse,  
Attorney.

Patented Sept. 4, 1923.

1,466,738

# UNITED STATES PATENT OFFICE.

CHARLES S. MORSE, OF ROLAND PARK, MARYLAND, ASSIGNOR TO BALTIMORE TUBE COMPANY, INC., OF BALTIMORE, MARYLAND, A CORPORATION OF VIRGINIA.

## METHOD AND MEANS FOR BILLET CASTING.

Application filed July 2, 1921. Serial No. 482,031.

To all whom it may concern:

Be it known that I, CHARLES S. MORSE, a citizen of the United States, residing at Roland Park, in the county of Baltimore, State of Maryland, have invented a new and useful Method and Means for Billet Casting, of which the following is a specification.

My invention relates to billet casting. The object is to provide improved method and means for casting hollow billets. The invention has especially to do with the method and means for securing an automatic relative shifting longitudinal movement between the core and the billet, during the contraction of the latter, due to cooling of the metal of the billet, in order to prevent injury to the billet, which frequently occurs when the billet is permitted to cool and contract in the usual way directly upon a rigid and fixed core.

Heretofore it has been the practice to provide a yielding or collapsible core that will give sufficiently to permit the contraction of the billet without injury thereto. The method has also been employed of withdrawing the core by external means, before the billet has sufficiently contracted to cause injury thereto.

By the present method however, it is proposed to so associate the core with the mold and to so shape the core, and also to coat the same with a suitable lubricant, that the action of the billet, upon contracting, is to force a relative longitudinal movement between billet and core.

Referring to the drawings, which illustrate, merely by way of example, suitable means for effecting my invention:

Fig. 1 is a longitudinal section, showing the core and mold associated in initial, or pouring position, and also showing the metal forming the billet, in its initial position relative thereto.

Fig. 2 is a similar view of the billet and core showing the approximate relative position of the billet and core after the cooling and consequent relative movement due to the contraction of the metal of the billet.

Similar numerals refer to similar parts throughout the several views.

In the example shown in the drawing the mold 5 is nearly cylindrical as to its inner wall. It is provided with the removable block 6, locked in place by the bolt 7. It is also preferably surmounted by the remov-

able pouring funnel 9. The core 8 is of tapered formation, that is, its cross-sectional dimension decreases constantly from one end to the other. In Fig. 1 it is shown with the smaller end extending downwardly toward or to the bottom of the mold or to the block 6. The core is also shown as provided with a coating 13, of suitable lubricating material such for example, as that formed by a mixture of flaked graphite and oil. This material being to a substantial degree heat resisting.

In operation, the mold and core are assembled substantially as shown in Fig. 1. The lower end of the core 8 extending downwardly to or near the bottom of the mold 5 or to the block 6. The upper end of the core is preferably centered by any suitable means such as the projections 10 connected with the removable funnel 9. The metal is poured by means of the funnel 9 into the annular space between the mold 5 and core 8 until molten metal rises in the mold to the required level, for example, that indicated by the dotted line 11. The metal thus poured into the mold about the core becomes the billet, marked 12.

As the billet 12 cools the metal contracts, and thus tends to become of slightly reduced cross-sectional dimension, that is, its periphery will become less, at any given point, than the adjacent periphery of the surrounding mold wall.

When this contraction of the billet takes place about a rigid and fixed core, it frequently happens that the contraction or shrinking not only causes such a tight engagement of billet and core that it is extremely difficult to remove the core from the billet, but also, the body of the billet will be cracked and thereby rendered useless.

I have discovered that by forming the core with a gradual but constantly diminishing cross-sectional dimension from one end to the other, and by coating the entire surface of the core that comes into contact with the metal of the billet, with a film or skin of suitable lubricating material; the billet, as it contracts upon the core, will, due to tapered formation of the core and the lubricating quality of the coating covering the core, cause a slight relative longitudinal movement between the billet and the core. That is to say, the reduced cross-sectional dimension of the inner periphery of the bil-

2  
let, at any point due to said contraction, will move to a correspondingly reduced cross-sectional peripheral dimension of the core due to said taper, and this relative movement between the billet and the core will correspond to the degree of contraction. This relative movement obviously need not be great, but will be sufficient to enable the billet, at any point in its circumference, to find a corresponding point in the core circumference where the reduced dimension of the core will compensate for the reduced dimension of the billet at said point due to said contraction. This relative movement between billet and core is of course, automatic, due to the force exerted by the contracting metal of the billet and facilitated by the inclined walls of the tapered core and by the lubricating effect of the coating applied thereto.

In the practice of the method above described I believe the best results are secured by arranging the elements with the small end of the core at or near the bottom of the mold as shown in the drawings so that the metal that first comes to rest in the mold, and consequently which begins to contract, is about the small end of the mold, while the metal above contracts progressively.

30 3. What I claim is:—

1. The method of casting hollow billets which consists in utilizing the inclined walls of a tapered core to secure an automatic relative longitudinal movement between billet and core due to the force exerted by the contraction of the billet.

2. The method of casting hollow billets which consists in utilizing the inclined walls of a tapered core to secure an automatic relative movement between billet and core due to the force exerted by the contraction of the billet, and facilitating said relative movement by a lubricating agent between the adjacent walls of billet and core.

45 3. The method of casting hollow billets which consists in utilizing the inclined walls of a tapered core to secure an automatic relative movement between billet and core due to the force exerted by the contraction of the billet, and facilitating said relative

of a lubricating agent between the billet and core.

4. The method of casting hollow billets which consists in utilizing the inclined walls of a tapered core to secure an automatic relative movement between billet and core due to the force exerted by the contraction of the billet, facilitating said relative automatic movement by utilizing the action of a lubricating agent between the billet and core, and so introducing the metal that the contraction will begin at the small end of the core.

5. In a billet casting device, the combination of a mold, and a cooperating tapered core, the parts so arranged and associated as to permit of relative automatic longitudinal movement between core and billet, the core having walls inclined sufficiently to enable the force developed by the contraction of the metal of the billet, cast about the core, to cause an automatic relative movement between billet and core during said contraction.

6. In a billet casting device, the combination of a mold, and a cooperating tapered core, the parts so arranged and associated as to permit of relative automatic movement between core and billet, the core having a lubricating agent applied thereto, and having walls inclined sufficiently to enable the force developed by the contraction of the metal of the billet, cast about the core, to cause an automatic relative movement between billet and core during said contraction.

7. In a billet casting device, the combination of a mold, and a cooperating tapered core, the parts arranged and associated with the small end of the core at the bottom of the mold, so as to permit of relative automatic movement between core and billet, and so that the metal that is poured shall first come to rest and begin to contract at the small end of the core, the core having a lubricating agent applied thereto, and having walls inclined sufficiently to enable the force developed by the contraction of the metal of the billet, cast about the core, to cause an automatic relative movement between billet and core during said contraction.

CHARLES S. MORSE.